

## UNITED STATES PATENT OFFICE

LAURI I. L. DURCHMAN, OF PETERSBURG, VIRGINIA

## PROCESS OF MANUFACTURING ALPHA CELLULOSE

No Drawing.

Application filed May 8, 1929. Serial No. 361,546.

My said invention relates to a new and useful method of manufacturing cellulose suitable for making of highgrade alphacellulose using the well known sulphate process with some alterations regarding used chemicals, cooking-time, temperature and pressure. The usual sulphate cooking process is a very drastic one by reason of the short cooking time and strong chemicals used, but for making kraftpulp it is satisfactory and commercial. For making an easy bleaching sulphate pulp with highest possible percentage of alphacellulose the chips, independent of what kind of wood is used, have to be digested under certain conditions of time, temperature and pressure with a composition of white and black liquors. As is well known, in the usual sulphate process the cooking proceeds for about three to three and one-half hours. According to my process cooking proceeds for from three to six hours. To prevent an oxidation of the fiber a certain amount of sodium sulphite ( $Na_2SO_3$ ) between 0.8-1.0% based on the air dry weight of the chips has to be added. This amount of  $Na_2SO_3$  is necessary if the  $Na_2S$  in the white liquor is lower than 30-35 gr. per liter. If the digesting operation has been a careful one the percentage of alphafiber may be found between 90-95%.

Thus obtained easy bleaching sulphate cellulose contains a large amount of incrusting matters and has a color various from pale yellow to dark brown. To bleach this pulp an excess of bleaching liquor would be necessary and the cellulose would not have the necessary whiteness and the percentage of alphacellulose would decrease too. The pulp has therefore to be given a treatment prior to the bleaching treatment which will remove, decompose and transfer incrusting matters into water soluble compounds. I have found that with boiling the cellulose in an open tank, or under pressure and using 2-6% of  $NaOH$ , or wash water with the same amount of  $NaOH$  from the strong caustic treatment which will be described later, and 2-6% of common salt ( $NaCl$ ) based on the dry weight of the cellulose under certain conditions of tempera-

ture and time a very easy bleaching cellulose can be obtained. The boiling time in an open tank is between three and six hours. The alkaline salts react with the incrusting substances partly dissolving and partly decomposing them into watersoluble compounds. After the cellulose has been thoroughly washed and thickened it is bleached. 55

The alkaline bleaching solution which contains from  $\frac{1}{4}$  to  $\frac{3}{4}\%$  of  $NaOH$  based upon the amount of bleaching powder used and which is added to the dry bleaching powder before adding water gives a somewhat slower bleaching but results in a highgrade bleached cellulose. The presence of alkali prevents a too quick bleaching and dissolves incrusting substances. A multiple stage bleaching operation is preferable because it gives a very satisfactory bleaching result, with a considerably smaller loss in the alphacellulose percentage. The first stage is a chlorination of the incrusting matters and the second stage a dissolving of the incrusting and coloring matters. It is of great advantage to take  $\frac{2}{3}$  of the necessary total bleaching solution into the first stage of bleaching. After the chlorine is exhausted and the cellulose thoroughly washed the second part or the last  $\frac{1}{3}$  is added. The temperature can be raised after 2 to 3 hours of 70

bleaching to  $40-45^{\circ}C$ . After the bleaching is finished the cellulose is thoroughly washed and thickened to highest possible dryness, and then the strong alkaline treatment with  $NaOH$  solution is given for about 5 hours at about room temperature. Bleached cellulose as above mentioned has after the bleaching 89-92% of alphacellulose. Depending upon the grade of desired percentage of alphacellulose in the finished pulp, the strength of the  $NaOH$  solution is based. Using a solution with 5-12% of  $NaOH$  under certain time, temperature and consistency an alphacellulose as high as 99% can be obtained. To recover the caustic liquor the cellulose has to be centrifuged and the first and second washwater saved for reuse (for the first boiling treatment) or to be taken for recovery with the black liquor. 95 100

The strong caustic liquor can be reused by adding fresh caustic to it.

After the cellulose has been washed with hot water and treated with a weak acetic acid solution it is washed and thickened, the acetic acid being preferably added to the hot water.

To meet the specifications for alphacellulose for using it in the manufacturing of rayon, lacquers, explosives, films, etc. the cellulose has to be given an oxalic acid treatment with 6-8% of oxalic acid based on the dry weight of the cellulose, which precipitates the main compound calcium, into calcium oxalate and dissolves the iron the treatment being continued for 3 to 5 hours at about room temperature. The oxalic acid can be recovered to about 80-90% if the cellulose is centrifuged. Thus recovered oxalic acid has to be filtered and strengthened up with fresh oxalic acid and can be reused. A very thorough washing after the oxalic treatment is necessary because the fiber has a great affinity to absorb alkaline and acid salts and precipitates.

My preferred process may be illustrated in a flow sheet as follows:

*Flow sheet*



Having thus fully described my said invention, what I claim as new and desire to secure by Letters Patent, is:

1. A process for producing easy bleaching cellulose which consists in cooking wood chips with black and white sulphate liquor with the addition of sodium sulphite in the proportion of 0.8-1.0% based on the airdry weight of the wood chips, continuing the cooking for a longer period than is the usual practice in the sulphate process, thereby increasing the alphacellulose content, and treating the pulp with a solution containing 2-6% sodium hydroxide and 2-6% common salt.

2. A process for producing easy bleaching cellulose which consists in cooking wood chips with black and white sulphate liquor with the addition of sodium sulphite in the proportion of 0.8-1.0% based on the airdry

weight of the wood chips and continuing the cooking for a longer period than is the usual practice in the sulphate process, and boiling the resultant pulp under atmospheric pressure with a solution containing 2-6% sodium hydroxide and 2-6% of common salt.

3. A process for producing alphacellulose which consists in cooking wood chips with black and white sulphate liquor with the addition of sodium sulphite in the proportion of 0.8-1.0% based on the airdry weight of the wood chips, boiling the resultant pulp under atmospheric pressure with a mixture containing 2-6% sodium hydroxide and 2-6% common salt, bleaching, and treating the bleached pulp at room temperature for three to six hours with a 5-12% solution of sodium hydroxide.

4. A process for producing alphacellulose which consists in cooking wood chips with black and white sulphate liquor with the addition of sodium sulphite in the proportion of 0.8-1.0% based on the airdry weight of the wood chips, boiling the resultant pulp under atmospheric pressure with a mixture containing sodium hydroxide and common salt, bleaching, treating the bleached pulp at room temperature for three to six hours with a 5-12% solution of sodium hydroxide, recovering the sodium hydroxide, washing, and treating with oxalic acid to neutralize the residual alkali and to facilitate extraction of other residual and coloring impurities.

In testimony whereof I affix my signature.

LAURI I. L. DURCHMAN.